

Sept. 7, 1948.

F. P. ALLES

2,448,507

PHOTOGRAPHIC ELEMENTS HAVING ANTIHALATION LAYER COMPOSED  
OF VINYL PYRIDINE POLYMER WITH VINYL PYRIDINE POLYMER  
SUBLAYER AND OUTER PROTECTIVE LAYER

Filed Aug. 1, 1946

FIG. 1.



FIG. 2.



INVENTOR.

FRANCIS PETER ALLES

BY

*Lynn Barratt Morris*

ATTORNEY

## UNITED STATES PATENT OFFICE

2,448,507

## PHOTOGRAPHIC ELEMENTS HAVING ANTI-HALATION LAYER COMPOSED OF VINYL-PYRIDINE POLYMER WITH VINYL-PYRIDINE POLYMER SUBLAYER AND OUTER PROTECTIVE LAYER

Francis Peter Alles, North Plainfield, N. J., assignor to E. I. du Pont de Nemours &amp; Company, Wilmington, Del., a corporation of Delaware

Application August 1, 1946, Serial No. 687,709

5 Claims. (Cl. 95—9)

1

This invention relates to photographic elements and, more particularly, to photographic elements bearing a novel, removable, antihalation layer on the reverse side. Still more particularly it relates to photographic elements which have a light-sensitive layer on one side of a support which transmits actinic light and the other side of the support has a composite structure consisting of a colloid layer and an antihalation layer wherein the binding agent is composed of a vinylpyridine polymer and an antiabrasion layer for said antihalation layer.

An object of this invention is to provide new and useful photographic elements which have removable antihalation layers. Another object is to provide such elements wherein the layers do not come off during alkaline development of the exposed element. A further object is to provide such elements wherein the antihalation layer can be readily removed in a weak acid-containing bath. A still further object is to provide such elements which are free from stain after removal of the antihalation coating. Another object is to provide antihalation layers which do not deleteriously affect the sensitivity of silver halide emulsion layers. Yet another object is to provide a composite antihalation photographic element which does not deteriorate or become tacky on storage. Still other objects will be apparent from the following description of the invention.

In a copending application of David Malcolm McQueen and Clay Weaver, Serial Number 687,708, filed on even date herewith, it is disclosed that the vinylpyridine polymers are eminently well-suited as the film-forming binding agent for the antihalation layer of a photographic element. The layers are not dissolved by the alkaline developer or the water rinse baths used after development. However, they are solubilized by the acid present in and at the concentration usually employed in the ordinary acid photographic processing baths, such as stop baths, acid fixing baths, acid hardening fixing baths, acid bleach baths, reversal bleach baths, etc. The vinylpyridine polymers are readily removable because of such solubility. Moreover, they are removable in acid developing baths.

The vinylpyridine polymers can be made by polymerizing a monomeric vinylpyridine, e. g., alpha-, beta-, or gamma-vinylpyridine or a homologue thereof containing an alkyl radical of one to four carbon atoms in the pyridine ring, in a liquid medium by the aid of a polymerization catalyst. An organic solvent solution can be used if desired in which case inert organic solvents are

2

used. However, emulsion polymerization is quite useful and bulk polymerization methods are effective. The polymerization is preferably carried out in an aqueous mineral acid solution or medium in the presence of a peroxy compound catalyst at temperatures from about 20° to 50° C. for a period of ten or less to 200 or more hours. The proportion of mineral acid, e. g., hydrochloric or sulfuric, may vary over a fairly wide range, e. g., from 0.5 to 2.5 mols of acid per mol of vinylpyridine monomer. The resulting solution may be diluted with water and the solution added to a basic solution, e. g., aqueous sodium hydroxide, and the precipitated resin filtered, washed, and dried. A neutralizing agent can be present in the wash water.

The invention is not limited to the use of polyvinylpyridine, including the alkyl substituted polyvinylpyridines, as the binding agent for the antihalation materials because copolymers soluble in 1% aqueous acetic acid which contain up to 20% of another polymerizable vinyl or vinylidene compound having a single vinyl group ( $\text{CH}_2=\text{C}<$ ) are useful. Suitable compounds for copolymerization with a monomeric vinylpyridine are styrene, acrylic esters and amides, alpha-alkyl-substituted acrylic esters and amides, acrylonitriles and methacrylonitriles.

In making the copolymers there may be used such materials as methyl or ethyl acrylates; methyl, ethyl, isobutyl, and methoxyethyl methacrylates; methacrylamide and N-methylacrylamide; acrylonitrile and methacrylonitrile; styrene; vinyl naphthalene, and the like or mixtures of two or more of these compounds.

In a preferred aspect of the invention, the polymers of unsubstituted alpha- or 2-vinylpyridine or its interpolymers containing 1 to 10% of a different interpolymers monomer are used. Such polymers are nonwater-soluble, synthetic resins soluble in alcohols, e. g., methyl, ethyl, propyl, and butyl, and mixtures of such alcohols with ketones, e. g., acetone, methyl ethyl ketone, methyl propyl ketone, and methyl isobutyl ketone or in certain chlorinated hydrocarbons, e. g., trichlorethylene. They form clear, light-colored, non-tacky films or coatings which are readily and completely soluble in dilute aqueous acids, e. g., acetic, hydrochloric, sulfamic, sulfuric, phosphoric, and oxalic acids.

The novel photographic elements of this invention consist of a support which transmits actinic light and has a light-sensitive colloid silver halide emulsion layer on one surface thereof. The other surface has disposed thereon, in order, a layer composed of a vinylpyridine polymer having the

above characteristics, next an antihalation layer composed of such polymer which has intimately distributed therethrough an antihalation material which absorbs actinic light, and finally a protective layer. The latter layer may be composed of various film-forming materials. Among the useful materials there may be mentioned water- and alkali-soluble polymers and cellulose derivatives and alginates, e. g., polyvinyl alcohol, sodium cellulose glycolate, ethyl cellulose, methyl cellulose, cellulose acid phthalate, starch glycolate, and alginic acids and their water-soluble salts, e. g., alkali metal and ammonium alginates.

The preferred photographic elements of the invention consist of a support which transmits actinic light which carries on one surface thereof a light-sensitive colloid silver halide emulsion layer and on the other side, in order, a thin, clear, polyvinylpyridine sublayer, next an antihalation layer composed of polyvinylpyridine having dispersed therethrough an antihalation material, and finally an antiabrasion layer composed of casein. The resulting elements when constructed with a transparent photographic film base constitute commercially important "daylight loading" photographic films. These films after exposure can be developed and washed in the usual manner. The entire backing can be readily removed by treatment in an acid bath as described above.

It has been found that the sublayer of the vinylpyridine polymer aids considerably in the removal of the antihalation material. It prevents staining of the film base by particles of the antihalation material. It has been found that when this layer is omitted that it is often necessary to rub the surface of the film element in order to remove surface discoloration due to particles of antihalation material.

The protective or antiabrasion layer also improves the elements. It prevents the staining of the colloid silver halide layer when the elements are packaged in the form of rolls.

A practical method of making the novel antihalation photographic elements is as follows: The vinylpyridine polymer is dissolved in a water-insoluble alcohol, e. g., methanol and ethanol, etc., in an amount of about 0.25 to 20% by weight of the alcohol. The resulting solution is then coated onto the back surface of a photographic support, for instance, a transparent film base or a transparentized paper. The layer is dried by removal of the solvent, e. g., by drying in a current of warm air. Another batch of vinylpyridine polymer is dissolved in a water-miscible alcohol in an amount of 0.25 to 20% by weight of the alcohol and an antihalation material admixed therewith. Thus antihalation pigments or dyes may be added in the form of small particles and dispersed or milled into the solution. Water-tolerant or spirit-soluble dyes can be added from a solvent solution. The solution is then applied to or coated on the back of a film base by any of the conventional coating methods, e. g., coating from a hopper provided with a doctor blade, dipping, by transfer or beading rollers, spraying, etc., and the solvent allowed to evaporate. A layer in the order of 1 to 10 microns is generally sufficient. However, substantially thicker layers can be made if desired. A light-sensitive layer, e. g., a colloid silver halide emulsion layer, is then coated on the opposite side of the base.

The photographic elements referred to above

are illustrated in the accompanying drawing wherein:

Fig. 1 is a schematic cross-sectional view of a photographic film element bearing a vinylpyridine polymer sublayer, an antihalation layer, and a protective layer; and

Fig. 2 is a schematic cross-sectional view of a transparentized paper photographic element bearing a vinylpyridine polymer sublayer, an antihalation layer, and a protective layer.

Referring now more particularly to the drawing, the film paper 1 has composed on one surface thereof a colloid silver halide emulsion layer 2. The rear surface of the base is coated with 15 a thin layer 3 which is composed of a vinylpyridine polymer upon which there is deposited an antihalation layer 4, which is composed of a vinylpyridine polymer containing an antihalation material. The outer surface of the latter layer is provided with an antiabrasion layer 5.

The element of Fig. 2 consists of a transparentized paper base 6, which has composed on one surface thereof a colloid silver halide emulsion layer 7. The rear surface of said base is provided with a thin layer 8 which is composed of a vinylpyridine polymer. An antihalation layer 9 is coated on the latter layer. It is composed of a vinylpyridine polymer and an antihalation material. An antiabrasion layer 10 is coated on 30 said antihalation layer.

The nature of light-absorption characteristics of the antihalation material for the layer will, of course, depend upon the particular characteristics of the emulsion. They are added in sufficient amounts to form an effective density which will stop the passage of the undesired light rays. Halation of blue-sensitive and ortho-chromatic emulsions can be minimized by the use of black and red non-halation layers. Panchromatic emulsions, theoretically, require black non-halation layers, although green and deep blue can be used advantageously. Natural occurring pigments of the above-mentioned colors may be used by this invention since the entire non-halation 45 coating is removed during processing. Metallo-dye complexes and inorganic, colored compounds are likewise suitable if they are of appropriate colors.

The invention will be further illustrated but 50 is not intended to be limited by the following example. The parts are by weight.

#### Example

A cellulose acetate film base was coated on the 55 back surface with a 1.25% solution of polymerized 2-vinylpyridine in methanol to a thickness of approximately one micron and dried. A 3% solution of carbon black-polyvinylpyridine in the ratio of 2.75 to 1 by weight in a methanol-ethanol mixture of equal parts by weight was 60 coated on the latter layer to a thickness of three microns. The particles of carbon black were milled into the solution by grinding in a ball mill for 20 hours. The antihalation coating was 65 over-coated with a solution of the following composition:

|                                   | Per cent |
|-----------------------------------|----------|
| Casein                            | 2.0      |
| Ammonium hydroxide (20% strength) | 2.5      |
| Distilled water                   | 25.0     |
| Methanol                          | 70.5     |

The daylight loading backing produced by the above procedure is easily and completely removed in weak acetic acid, there is no residual 75 smudge or staining of the base, mechanical

brushes or sponges are not required, and the backing does not become less soluble in acid on aging.

If it is desired to remove the antihalation layer before fixation, it may be solubilized by immersing the film in weak acid baths, e. g., acetic or citric acid baths, which are commonly employed as a stop bath between the development and fixation stages of processing.

In general, any dye or pigment which possesses the property of absorbing actinic light, of being readily dissolved or destroyed in ordinary photographic baths, and of not injuring such baths may be used. The dye or dyes to be used in any specific instance are primarily determined by the light-sensitivity of the emulsion. Such emulsions are usually gelatin silver halide emulsions which contain sensitizers, such as cyanine, carbocyanine, pseudo-cyanine, cyazine bases and salts. That is, it must be absorptive of light of the wavelengths to which the emulsion is sensitive. In general, the dye should be added in an amount sufficient to give a photographic density of 0.2 to 0.8 or the amount of dyed layer should be sufficient to give such a density. When added from ethanol, etc., a very fine subdivision of the dye in the layer is obtained. As examples of additional useful dyes, mention is made of:

Auramine (C. I. 655)  
 Helianthin (C. I. 142, 146)  
 Brilliant Yellow S (C. I. 144)  
 Chrysoin (C. I. 148)  
 Acid Blue Black (C. I. 246)  
 Rhodamine (C. I. 749, 750, 751, 746, 753, 761, 763)  
 Fuchsin (C. I. 677)  
 Sufranine G (C. I. 841)  
 Ponceau 6R (C. I. 186)  
 Crocein Scarlet (C. I. 277, 251, 286, 252, 291, 183)  
 Azorubin (C. I. 179)  
 Sufranine O (C. I. 841)  
 Ponceau 2R (C. I. 79)  
 Spirit Solution Nigrosine (C. I. 864)  
 Metanil Yellow (C. I. 138)

The color index number (C. I.) referred to above are identified as follows: "Society of Dyers & Colourists Colour-Index, edited by F. M. Rowe, D. Sc., F. I. C., First Edition January 1924, published by The Society at the General Offices, 30 Pearl Assurance Buildings, Bradford, Yorkshire."

The invention is not limited to the use of cellulose ester film bases but may be used with practically any transparent film. The polyvinylpyridine layers are adherent to various other film materials, e. g., polyamides, cellulose nitrate, polyvinyl acetals, cellulose propionate, cellulose mixed esters, cellulose ethers, vinyl chloride and copolymers, styrene, acrylonitrile and copolymers, polyesters, vinyl acetate and copolymers, vinyl fluoride and copolymers, polyvinyl alcohol, transparentized paper, etc.

This invention has the advantage that a non-tacky antihalation layer which is insoluble in water or alkaline solutions but is readily soluble in dilute acid baths may be quickly prepared. A further advantage is the fact that stable, non-tacky, non-reactive, antihalation layers may be easily prepared. Thus films may be tightly rolled up with the antihalation layer in direct contact with the emulsion layer and stored for long periods of time without any detrimental effects.

As many widely different embodiments of this invention can be made without departing from the spirit and scope thereof, it is to be understood that the invention is not to be limited except as defined by the claims.

What is claimed is:

1. A photographic element comprising a support which transmits actinic light, a light-sensitive colloid silver halide emulsion layer on one surface of said support and on the other surface of said support, in order, a clear layer composed of a water-insoluble vinylpyridine polymer which is soluble in 1% aqueous acetic acid, an antihalation layer composed of such a vinylpyridine polymer which is soluble in 1% aqueous acetic acid and contains an antihalation material, and an antiabrasion layer composed of a water-soluble film-forming material.

2. A photographic element comprising a support which transmits actinic light, a light-sensitive colloid silver halide emulsion layer on one surface of said support and on the other surface of said support, in order, a clear layer composed of a water-insoluble vinylpyridine polymer which is soluble in 1% aqueous acetic acid, an antihalation layer composed of such a vinylpyridine polymer which is soluble in 1% aqueous acetic acid and contains an antihalation material, and an antiabrasion layer composed of casein.

3. A photographic film element comprising a transparent film base, a light-sensitive colloid silver halide emulsion layer on one surface of said film base and on the other surface of the film base, in order, a clear polyvinylpyridine layer, an antihalation layer consisting of polyvinylpyridine which contains an antihalation material, and an antiabrasion layer composed of a water-soluble film-forming material, said polyvinylpyridine being water-insoluble but soluble in 1% aqueous acetic acid.

4. A photographic film element comprising a transparent film base, a light-sensitive colloid silver halide emulsion layer on one surface of said film base and on the other surface of the film base, in order, a clear 2-vinylpyridine polymer layer, an antihalation layer consisting of 2-vinylpyridine polymer which contains an antihalation material, and an antiabrasion layer composed of a water-soluble, film-forming material, said 2-vinylpyridine polymer being water-insoluble but soluble in 1% aqueous acetic acid.

5. A photographic film element comprising a transparent film base, a light-sensitive colloid silver halide emulsion layer on one surface of said film base and on the other surface of the film base, in order, a clear 2-vinylpyridine polymer layer, an antihalation layer consisting of 2-vinylpyridine polymer which contains an antihalation material, and an antiabrasion layer composed of water-soluble casein, said 2-vinylpyridine polymer being water-insoluble but soluble in 1% aqueous acetic acid.

FRANCIS PETER ALLES.

#### REFERENCES CITED

The following references are of record in the file of this patent:

#### UNITED STATES PATENTS

| Number    | Name    | Date          |
|-----------|---------|---------------|
| 1,939,171 | Hickman | Dec. 12, 1933 |
| 2,182,794 | Dawson  | Dec. 12, 1939 |